

## UNITED STATES PATENT OFFICE

2,205,120

PROCESS FOR RENDERING CELLULOSE-  
CONTAINING MATERIAL CREASE-RESIST-  
ANT AND PRODUCTS OBTAINED THEREBY

George Heberlein, Jr., Ernst Weiss, and Hans  
Hemmi, Wattwil, Switzerland, assignors to  
Heberlein Patent Corporation, New York, N. Y.,  
a corporation of New York

No Drawing. Application December 23, 1937, Se-  
rial No. 181,454. In Germany December 28,  
1936

11 Claims. (Cl. 8—116)

This invention relates to processes for rendering cellulosic textile materials wrinkle-resistant and also to products therefrom.

It has previously been found in accordance with the application of Frauenfelder, Ser. No. 62,994, filed February 8, 1936, that a good resistance to wrinkling in cellulosic material such as cotton and other natural cellulose-containing fibers, as well as regenerated cellulose, artificial silk fibers such for example as viscose and cuprammonium can be produced without deposition of an artificial resin within or on the fiber by treatment with formaldehyde and a suitable catalyst. According to this prior process fabrics, yarns and unspun fibers of materials mentioned above were preferably steeped in an aqueous solution of formaldehyde of proper strength which contained a catalyst of a non-alkaline character, and, if necessary, were centrifuged or rung out and thereupon heated while substantially dry to a temperature of about 90°-160° C. The materials treated according to this process not only were wrinkle-proof but showed an almost complete freedom from shrinkage. This prior process resulted in some decrease of the strength of the materials treated.

We have found in accordance with the present invention that cellulose-containing material can be made crease-resistant and its strength substantially maintained by treating it with a swelling agent and thereafter with formaldehyde in the presence of a non-alkaline catalyst, and heating while dry to a temperature of about 90° C. to about 160° C. for a sufficient length of time to produce an effective wrinkle-resistance. During the treatment with the swelling agent we have also found that further improvement in the strength and other valuable properties may be given to natural cellulose fiber, for example such as cotton, by giving it a caustic swelling and shrinking and then stretching it preferably beyond its original length, and thereafter proceeding with the wrinkle-resistant treatment. We have also found that improved effect yarns may be made in accordance with our invention.

The principal object of the invention accordingly is to produce a simple efficient process of the kind described and to produce a series of improved products thereby.

The invention comprises the novel products as well as the novel processes and steps of processes according to which such products are manufactured, the specific embodiments of which are described hereinafter by way of example and in

accordance with which we now prefer to practice the invention.

We have found that the invention can be carried out in a simple and effective manner by exposing the goods before the wrinkle-resistant treatment to the action of a swelling agent, leaving the goods a short time in such condition, then thoroughly washing out the swelling agent and then treating them, in the manner above referred to, with formaldehyde in the presence of a non-alkaline catalyst and heating them for a sufficient length of time to about 90° C. to about 160° C. to produce the desired crease-resistance. The surprising fact has been noted accordingly in so carrying out our process that it is not only possible to improve the strength of the goods but in addition to this if the goods so treated by pre-swelling and formaldehyde are thereafter treated with various swelling agents, they show an improved resistance thereto. Thus for instance the breaking elongation of rayon is improved and at the same time the tensile strength may be increased beyond the tensile strength of the untreated material. The breaking elongation and tensile strength of cotton is also improved by the process. Resistance to swelling agents for example is shown by the following: If parchmentizing sulfuric acid is allowed to act on the goods for more than one minute or mercerizing lye (caustic soda) is allowed to act for several hours, no shrinking or other change is noticeable. We have also found that material treated in accordance with the invention is almost completely immune to substantive dyestuffs.

All of the known swelling agents may be employed for the carrying out of preliminary treatment in accordance with our invention. For instance alkalis, such as caustic soda solution, caustic potash solution, quaternary ammonium bases, various acids, such as sulfuric acid, phosphoric acid, etc. may be employed. Salt solutions, such as calcium rhodanide, zinc chloride, ammoniacal copper oxide and others may be used. However, caustic alkalis appear to be especially suitable, particularly caustic soda solution. These excel because of their low price and particularly because of good results which they give in increasing the breaking elongation, tensile strength and resistance to swelling agents of the completed material.

In treating various textile materials there must be taken into consideration in each individual case the special nature of the material to be treated. Artificial silk (rayon) is preferably swelled with caustic potash solutions. A notice-

able effect can be observed at a strength of 2° Bé. while for good results concentrations of 6° Bé. or more are required. Concentrations of up to even higher than 30° Bé. can be applied, if desired. Caustic soda solution may also be used provided concentrations are employed which will not cause injury to the rayon. Good results can be obtained with a caustic soda lye of about 3° Bé. but higher concentrations may be applied if desired. It is advisable to subject the rayon for a number of minutes in untensioned condition to the action of the swelling agent, then to wash thoroughly, if necessary, with hot water and to follow this, with or without intermediate dyeing, by the formaldehyde treatment. Normally the swelling agent is used at room temperature, but higher and lower temperatures may also be used.

In the case of cotton goods results may be obtained with concentrations of the swelling agents which are higher than the lower limits which can be used for rayon. If one uses lye of mercerizing strength, one obtains an improved breaking elongation with moderate tensile strength if the goods are treated in loose condition and are allowed to shrink in the lye. A particularly good tensile strength is obtained if the goods, preferably in the form of yarn, are first caused to shrink under the action of the lye, to their minimum length, and thereupon are stretched. It has been found that the effect thus obtained is better than that produced by standard mercerizing treatment in which the yarn is kept uniformly under tension from the beginning of the treatment to the end.

In general in the case of cotton the tensile strength is greater, the more strongly the yarn impregnated with the swelling agent is thereafter stretched after complete shrinking. Stretchings even beyond the original length can be applied with good results. The swelling agent, especially caustic soda solution, can be applied in heated condition. Temperatures above 100° C. can be used but heated mercerizing liquors of about 50° C. and 30° Bé. appear to give an especially favorable result.

In the case of cotton it is advisable to clean the fiber prior to the treatment in accordance with the invention, for instance by kier boiling, scouring, etc. because in such a case there is a complete wetting through with the swelling agent and subsequently with formaldehyde where the latter is employed in solution. On the other hand it is not necessary to bleach the fibers before the treatment in accordance with the invention for the purpose of destroying the natural colors contained therein by means of hypochlorite, peroxide of hydrogen, etc., although such bleaching may be practised, if desired.

The resistance to swelling agents referred to above is of special importance if the process of the invention is applied to yarns and these yarns are thereupon woven as effects in a fabric otherwise consisting of untreated fiber material. The finished fabric, which for instance may consist on the one hand of raw cotton yarn and on the other hand of cotton yarn or rayon yarn treated in accordance with our invention as effect yarns, can be scoured (kier boiled) and bleached without difficulty and without losing the valuable resist properties of the effect yarns. If the fabric containing effect yarns treated as just mentioned is then treated by one of the known finishing processes, such as mercerizing without tensioning, treatment with sulfuric acid having a shrinking

parchmentizing action or other known swelling agents, the effect yarns remain unchanged while the other yarns in the manner known per se and depending on the kind of finishing liquor or bath, shrink, become stiff, transparent or the like. As further fibrous materials suitable for treatment by the swelling agent for preparing such fabrics in which the effect yarns are woven, we may employ other cellulose-containing yarns such as rayon, linen, cell-wool (viscose spun rayon) or the like, and also animal fibers.

The following are specific examples of the process as we now prefer to practice it. It is to be understood that these examples are simply illustrative and that the invention is not limited thereto except as indicated in the appended claims.

#### Examples

1. Cotton yarn in skeins is normally mercerised with caustic soda of 32° Bé. in a yarn mercerizing apparatus. It is then washed out with hot and cold water and dried. Thereupon the yarn is impregnated in a bath containing 56 liters of water, 40 liters of formaldehyde 40% and 40 liters of solution of aluminium sulphocyanide of 17° Bé. It is then centrifuged and dried during several hours at 50–60° C. After this it is heated during a quarter of an hour at 120–125° C. and finally, to eliminate the odour of formaldehyde, washed out with a diluted solution of soap or ammonia in water, rinsed and dried.

2. Cotton yarn, the same as above, are treated following Example 1 with the exception that instead of normally mercerizing it is stretched just beneath the tearing-limit during the mercerisation.

The tensile strength of the overstretched mercerized yarn is about 20% higher than the tensile strength of the normally mercerized yarn and is of the same range or beyond the range of the unmercerized untreated preliminary material. The material so treated shows a higher orientation in its micelles.

3. Viscose-yarn is desized with a solution of 3 g. soap per liter and one of the usual textile assistants and then first washed with warm and subsequently with cold water and dried. Thereupon it is swelled in a loose condition with caustic potash of 6° Bé. during 5 minutes at 18–20° C., rinsed with boiling water, washed out with cold water and soured with sulphuric acid of 0.8° Bé., washed and dried. The yarn is then treated with the same impregnating bath as described above in Example 1 during 10 minutes, centrifuged and dried during several hours. After this it is heated during 20 minutes at 118–120° C. For deodorization it may then be rinsed with a diluted soap- or ammonia-solution, washed out and dried.

The breaking elongation of the so-treated viscose-yarn is about 25% higher than the breaking elongation of a formaldehyde-treated yarn which had not been swelled before, whereas the tensile strength is about of the same range or beyond the tensile strength of the untreated preliminary material.

In the appended claims where the expression "cellulose-containing material" or "cellulose-containing fabric" or the like expressions are used, they are employed to cover cotton or other natural cellulose-containing fibers, as well as all regenerated-cellulose-artificial silks for example such as viscose and cuprammonium silk; and in the form of fibers, yarn or fabric, either used alone or in combination with other fibers. In

5 the process claims where the expression "formaldehyde" is used, it is intended to include polymers of formaldehyde and formaldehyde-splitting compounds. Where the expression "non-alkaline catalyst" is used it is employed to cover acid catalysts, substances liberating an acid catalyst in solution or when exposed to the reaction conditions here described in which latter case they may also be neutral in the original state,

## 10 but not alkaline catalysts.

15 While the invention has been described in detail with respect to particular preferred examples, it will be understood by those skilled in the art after understanding the invention that various changes and further modifications may be made without departing from the spirit and scope of the invention and it is intended therefore in the appended claims to cover all such changes and modifications.

20 What is claimed as new and desired to be secured by Letters Patent is:

25 secured by Letters Patent, as:  
1. A process for rendering cellulose-containing  
material crease-resistant which comprises treat-  
ing cellulose-containing material with a swelling  
agent, thereafter impregnating the material with  
formaldehyde in the presence of a non-alkaline  
catalyst, heating the impregnated material while  
substantially dry for a sufficient length of time  
to about 90-160° C. and causing a chemical com-  
30 bination between the cellulose and formaldehyde  
whereby an effective crease-resistant quality is  
obtained and the tendency of the formaldehyde  
to weaken the fiber is at least in part offset by  
the preswelling.

35 2. A process for rendering cellulose-containing  
material crease-resistant which comprises treat-  
ing cotton with caustic alkali of mercerizing  
strength, thereafter impregnating the material  
with formaldehyde in the presence of a non-  
40 alkaline catalyst, heating the impregnated ma-  
terial while substantially dry for a sufficient  
length of time to about 90-160° C. and causing a  
chemical combination between the cellulose and  
formaldehyde whereby an effective crease-resist-  
45 ant quality is obtained and the tendency of the  
formaldehyde to weaken the fiber is at least in  
part offset by the preswelling.

3. A process according to claim 1 in which the swelling agent is applied at a temperature of the order of 50-100° C.

4. A process according to claim 2 in which the mercerizing agent is at approximately 50° C. or above and the mercerizing liquor is of approximately 30° Bé.

## 55 5. A process for rendering cellulose-containing

material crease-resistant which comprises treating artificial silk with caustic potash of swelling strength, thereafter impregnating the material with a crease-resistant agent which consists principally of formaldehyde in the presence of a non-alkaline catalyst and heating the impregnated material while dry for a sufficient length of time to about 90-160° C. whereby an effective crease-resistant quality is obtained.

6. A process for rendering cellulose-containing material crease-resistant which comprises treating cotton with a swelling agent, thereby shrinking the cotton, then stretching the cotton, thereafter impregnating the material with a crease-resistant agent which consists principally of formaldehyde in the presence of a non-alkaline catalyst and heating the impregnated material while dry for a sufficient length of time to about 90-160° C. whereby an effective crease-resistant quality is obtained. 10 15 20

7. A process according to claim 6 in which the cotton is first swollen and shrunk with caustic alkali of mercerizing strength and then stretched so that it has a greater length than it had prior to the treatment with the caustic alkali.

8. A process for rendering cellulose-containing material crease-resistant which comprises subjecting cotton to a mercerizing alkali treatment thereby mercerizing and shrinking it, stretching the cotton to beyond its original length while 30 washing it to remove the alkali, then impregnating the cotton while still in the stretched condition with formaldehyde in the presence of a non-alkaline catalyst and heating the impregnated material while dry for a sufficient length 35 of time to about 90-160° C. thereby giving to the cotton an effective crease-resistant quality and improved strength.

9. As a new product, a substantially shrink-proof cellulose-containing material swollen with a swelling agent and thereafter chemically combined with formaldehyde, said product having a strength substantially higher than such material treated with formaldehyde without the preliminary swelling treatment. 40

10. A new product in accordance with claim 9 in which the swelling agent employed is an alkaline mercerizing agent.

11. A new product in accordance with claim 9 in which the cellulose-containing material is cotton having a high orientation in its micelles. 50

GEORGE HEBERLEIN, JR.  
ERNST WEISS  
HANS HEMMI.